



US005482913A

# United States Patent [19]

Satake et al.

[11] Patent Number: 5,482,913

[45] Date of Patent: Jan. 9, 1996

## [54] RECORDING SHEET

[75] Inventors: **Toshimi Satake; Tomoaki Nagai; Toshiyuki Takano; Akio Sekine**, all of Tokyo, Japan[73] Assignee: **Nippon Paper Industries, Co., Ltd.**, Tokyo, Japan[21] Appl. No.: **166,815**[22] Filed: **Dec. 15, 1993**

## [30] Foreign Application Priority Data

Dec. 17, 1992 [JP] Japan ..... 4-336472

[51] Int. Cl.<sup>6</sup> ..... **B41M 5/30**[52] U.S. Cl. ..... **503/210**; 430/200; 430/201; 503/211; 503/212; 503/216; 503/225

[58] Field of Search ..... 427/150-152; 503/216, 217, 225, 210-212; 430/200, 201, 180

## [56] References Cited

## U.S. PATENT DOCUMENTS

4,439,512 3/1984 Ceintrey ..... 430/180

## FOREIGN PATENT DOCUMENTS

0520404 12/1992 European Pat. Off. ..... 503/216  
2655184 6/1977 Germany ..... 503/216  
60-184879 9/1985 Japan ..... 503/216

## OTHER PUBLICATIONS

Chemical Abstracts, vol. 118, No. 18, 3 May 1993, Columbus, Ohio, abstract No. 180127, p. 782 &amp; JP-A-4-310 790 (Mitsubishi Paper Mills).

Patent Abstracts Of Japan vol. 10, No. 29 (M-451) (2086)

5 Feb. 1986 &amp; JP-A 60-184 879 (Mitsubishi Seishi). Chemical Abstracts, vol. 107, No. 8, 24 Aug. 1987, Columbus, Ohio, abstract No. 68275b, p. 617; JP-A-61 293 889 (Fuji Photo Film Co.).

Chemical Abstracts, vol. 116, No. 20, 18 May 1992, Columbus, Ohio, abstract No. 204609d, p. 716 &amp; JP-A-3 253 390 (Nicca Chemical Co.).

Jerry March 'Advanced Organic Chemistry 2. edition' McGraw-Hill, Tokyo 1977.

Abstract of Japanese laid-Open Publication 60-34892. Feb. 1985.

Abstract of Japanese Laid-Open Publication 60-184879. Sep. 1985.

Abstract of Japanese Laid-Open Publication 60-210491. Oct. 1985.

Abstract of Japanese Laid-Open Publication 63-137888. Jun. 1988.

Abstract of Japanese Laid-Open Publication 4-117351. Apr. 1992.

Abstract of Japanese Laid-Open Publication 4-144787. May 1992.

*Primary Examiner*—B. Hamilton Hess*Attorney, Agent, or Firm*—Sherman and Shalloway

## [57] ABSTRACT

A dispersion of a carbonate type blocked color developer having a hydroxyl group having a color developing function which is blocked by an O-substituted oxycarbonyl group (—(C=O)OR<sub>1</sub>), and a metal salt of an organic acid or inorganic acid or a leuco dye are mixed to obtain an opaque undeveloped coating color, and the coating color is coated on paper or the like to obtain a recording sheet. Also, the coating color is further mixed with a light absorbent to obtain an opaque undeveloped coating color, which is coated on paper or the like to obtain an optical recording sheet.

19 Claims, No Drawings

**1**  
**RECORDING SHEET**

**FIELD OF THE INVENTION**

This invention relates to a thermal recording sheet which is capable of recording by way of heat or light.

**DESCRIPTION OF THE PRIOR ART**

Thermal recording sheets used for facsimiles or the like comprise an opaque substrate such as paper coated thereon with coating color obtained by mixing and finely dispersing a colorless or pale colored electron-donating dye and a color developer in an aqueous solution of a water-soluble binder. However, these thermal recording sheets have been defective in that they tend to fog in undeveloped portions when stored in a high-temperature place or coming in contact with a solvent.

With the aim of eliminating such a disadvantage, Japanese Patent Publication Laid-open (Japanese OPI) 52-76118, Japanese OPI 60-184879, Japanese OPI 60-210491, Japanese OPI 63-137888, Japanese OPI 4-117351, and Japanese OPI 4-144787 disclosed a thermal recording material or a thermal recording sheet containing a urethane-type blocked color developer obtained by reacting a phenolic compound with an isocyanate compound.

These urethane-type blocked color developers are inactive at room temperature because a hydroxyl group having a color-developing function is chemically blocked but, when heated, decompose to the original color developer and the isocyanate compound to cause an electron-donating dye such as a leuco dye to develop a color. Therefore, a recording sheet using the color developer of this type does not develop a color unless a decomposition temperature is reached, nor does develop an unnecessary color (fogging) by heat or solvents.

Furthermore, Japanese OPI 60-34892 discloses use of a carbonate compound as a sensitizer.

However, recording sheets using a urethane-type blocked color developer have involved a problem in safety, because the color developer forms an isocyanate compound when decomposed by heating to develop a color, and have been insufficient in sensitivity.

Further, a carbonate compound is used merely as a sensitizer in combination with a color developer, and it has been unknown that a carbonate compound alone is used as a color developer.

**OBJECT OF THE INVENTION**

With a view to solve the above problems, a primary object of the present invention is to provide a recording sheet using a carbonate-type blocked color developer.

**SUMMARY OF THE INVENTION**

In accordance with the present invention, there is provided a recording sheet comprising an opaque recording layer containing a color developer of Formula (1) in which at least one of phenolic hydroxyl groups having a color-developing function is blocked by an O-substituted oxy carbonyl group ( $-(C=O)OR_1$ ), and a metal salt of an organic acid or a metal salt of an inorganic acid or a leuco dye which reacts with the color developer to develop a color.

**2**



(wherein R denotes a substituted or unsubstituted  $C_6-C_{30}$ -aromatic ring.  $R_1$  is substituted or unsubstituted  $C_1-C_{18}$ -alkyl group, substituted or unsubstituted  $C_3-C_{15}$ -cycloalkyl group, substituted or unsubstituted  $C_1-C_{12}$ -halogenated alkyl group, substituted or unsubstituted  $C_1-C_{12}$ -alkoxy-alkyl group, substituted or unsubstituted  $C_1-C_{12}$ -silylalkyl group, vinyl group, allyl group, substituted or unsubstituted  $C_7-C_{18}$ -aryl alkyl group, substituted or unsubstituted  $C_{13}-C_{25}$ -diphenyl methyl group, substituted or unsubstituted  $C_{19}-C_{35}$ -triphenyl methyl group, substituted or unsubstituted  $C_6-C_{20}$ -aryl group, or substituted or unsubstituted  $C_{10}-C_{20}$ -naphthyl group, except 2,3,5-trimethylphenyl group, p-tert-butylphenyl group, and xylyl group. a and b are integers from 1 to 3, and a  $\geq b$ , provided, however, that a case is excepted where a-b-1 and a combination of R and  $R_1$  is phenyl group and xylyl group, phenyl group and p-tert-butylphenyl group, phenyl group and p-diphenyl group, phenyl group and naphthyl group, or phenyl group and p-methoxycarbonylphenyl group.)

The color developer of Formula (1) used in the present invention, that is, a carbonate-type blocked color developer, can be produced by the following methods:

A first method is to add an alkyl chloroformate or an aryl chloroformate to a phenolic compound as a color developing compound in the presence of a base:



For example, when 4-hydroxy-4'-isopropylxydiphenyl sulfone is reacted with ethyl chloroformate in the presence of pyridine, a compound (12) can be obtained.

In a second method, a phenolic compound as a color developer is converted to an aryl chloroformate using phosgene or trichloromethyl chloroformate, and then an alcohol or phenol is added to the aryl chloroformate.



Aryl chloroformates derived from phenolic compounds include the following:



-continued



A third method is to react a dialkyldicarbonate compound with a phenolic compound as a color developer in the presence of a base:



For example, when bisphenol S is reacted with di-tert-butyl dicarbonate in the presence of pyridine, a compound (20) can be obtained.

Phenolic compounds to be carbonated are: for example phenol, o-methylphenol, m-methylphenol, p-methylphenol, p-methoxyphenol, p-nitrophenol, p-chlorophenol, p-bromophenol, 3,4-dichlorophenol, p-tert-butylphenol, p-phenylphenol, 3-diethylaminophenol, 1-naphthol, 2-naphthol, methyl p-hydroxybenzoate, ethyl p-hydroxybenzoate, propyl p-hydroxybenzoate, isopropyl p-hydroxybenzoate, butyl

p-hydroxybenzoate, benzyl p-hydroxybenzoate, 4-hydroxy-4'-isopropoxydiphenyl sulfone, 4-methyl-4'-hydroxydiphenyl sulfone, 4-hydroxy-4'-chlorodiphenyl sulfone, 4-hydroxy-4'-n-butoxy diphenyl sulfone, salicylic acid, ethyl salicylate, catechol, resorcinol, tert-butylcatechol, p,p'-bibiphenol, 4,4'-thiodiphenol, bis(4-hydroxyphenyl) sulfone, 4-methyl-3',4'dihydroxydiphenyl sulfone, 3,3'-diallyl-4,4'-dihydroxydiphenyl sulfone, 1,1-bis(p-hydroxyphenyl) propane, 1,1-bis(p-hydroxyphenol) cyclohexane, 2,2-bis(p-hydroxyphenyl) propane, 1,3-propyleneglycoldi(p-hydroxybenzoic ester), 1,4-butyleneglycoldi(p-hydroxybenzoic ester), hexyleneglycoldi(p-hydroxybenzoic ester), ethyleneglycoldi(p-hydroxyphenylether), hexyleneglycoldi(p-hydroxyphenylether), methyl bis(4-hydroxyphenol)acetate, ethyl bis(4-hydroxyphenyl)acetate, phenyl bis(4-hydroxyphenyl)acetate, pyrogallol, phloroglucinol, gallic acid, methyl gallate, ethyl gallate, n-propyl gallate, isoamyl gallate, lauryl gallate, and stearyl gallate.

The O-substituted oxycarbonyl group  $-(C=O)OR_1$  includes the following:

- |                                                                                     |                                              |
|-------------------------------------------------------------------------------------|----------------------------------------------|
| —(C=O)O—CH <sub>3</sub>                                                             | methoxycarbonyl                              |
| —(C=O)O—C <sub>2</sub> H <sub>5</sub>                                               | ethoxycarbonyl                               |
| —(C=O)O-n-C <sub>3</sub> H <sub>7</sub>                                             | n-propoxycarbonyl                            |
| —(C=O)O-iso-C <sub>3</sub> H <sub>7</sub>                                           | iso-propoxycarbonyl                          |
| 25   —(C=O)O-n-C <sub>4</sub> H <sub>9</sub>                                        | n-butoxycarbonyl                             |
| —(C=O)O-iso-C <sub>4</sub> H <sub>9</sub>                                           | iso-butoxycarboxyl                           |
| —(C=O)O-sec-C <sub>4</sub> H <sub>9</sub>                                           | sec-butoxycarbonyl                           |
| —(C=O)O-tert-C <sub>4</sub> H <sub>9</sub>                                          | tert-butoxycarbonyl                          |
| 30   —(C=O)O-n-C <sub>5</sub> H <sub>11</sub>                                       | n-amylloxycarbonyl                           |
| —(C=O)O-n-C <sub>6</sub> H <sub>13</sub>                                            | n-hexyloxycarbonyl                           |
| —(C=O)O-n-C <sub>7</sub> H <sub>15</sub>                                            | n-heptyloxycarbonyl                          |
| —(C=O)O-n-C <sub>8</sub> H <sub>17</sub>                                            | n-octyloxycarbonyl                           |
| —(C=O)O-n-C <sub>9</sub> H <sub>19</sub>                                            | n-nonyloxycarbonyl                           |
| —(C=O)O-n-C <sub>16</sub> H <sub>33</sub>                                           | n-hexadecyloxycarbonyl                       |
| 35   —(C=O)O-n-C <sub>6</sub> H <sub>11</sub>                                       | cyclohexyloxycarbonyl                        |
| —(C=O)O—CHClCH <sub>3</sub>                                                         | 1-chloroethoxycarbonyl                       |
| —(C=O)O—CH <sub>2</sub> CH <sub>2</sub> Cl                                          | 2-chloroethoxycarbonyl                       |
| —(C=O)O—CH <sub>2</sub> CH <sub>2</sub> CCl <sub>3</sub>                            | 2,2,2-trichloroethoxycarbonyl                |
| —(C=O)O—CH <sub>2</sub> CH <sub>2</sub> OCH <sub>3</sub>                            | 2-methoxyethoxycarbonyl                      |
| 40   —(C=O)O—CH <sub>2</sub> CH <sub>2</sub> OC <sub>2</sub> H <sub>5</sub>         | 2-ethoxyethoxycarbonyl                       |
| —(C=O)O—CH <sub>2</sub> CH <sub>2</sub> OC <sub>4</sub> H <sub>9</sub>              | 2-butoxyethoxycarbonyl                       |
| —(C=O)O—CH <sub>2</sub> CH <sub>2</sub> CH(OCH <sub>3</sub> )CH <sub>3</sub>        | 3-methoxybutoxy- carbonyl                    |
| 45   —(C=O)O—CH <sub>2</sub> CH <sub>2</sub> Si(CH <sub>3</sub> ) <sub>3</sub>      | 2-(trimethylsilyl)ethoxy- carbonyl           |
| —(C=O)O—CH <sub>2</sub> CH <sub>2</sub> SO <sub>2</sub> CH <sub>3</sub>             | 2-methylsulfonylethoxy- carbonyl             |
| —(C=O)O—CH=CH <sub>2</sub>                                                          | vinyloxycarbonyl                             |
| —(C=O)O—CH <sub>2</sub> CH=CH <sub>2</sub>                                          | allyloxycarbonyl                             |
| 50   —(C=O)O—CH <sub>2</sub> CH <sub>2</sub> OOCC(CH <sub>3</sub> )=CH <sub>2</sub> | 2-meth- acrylethoxycarbonyl                  |
| —(C=O)O—CH <sub>2</sub> C <sub>6</sub> H <sub>5</sub>                               | benzyloxycarbonyl                            |
| —(C=O)O—CH <sub>2</sub> C <sub>6</sub> H <sub>4</sub> NO <sub>2</sub>               | p-nitrobenzyloxycarbonyl                     |
| —(C=O)O—CH(CH <sub>3</sub> )C <sub>6</sub> H <sub>5</sub>                           | $\alpha$ -methylbenzyloxycarbonyl            |
| 55   —(C=O)O—C(CH <sub>3</sub> ) <sub>2</sub> C <sub>6</sub> H <sub>5</sub>         | $\alpha,\alpha$ -dimethylbenzyloxycarbo- nyl |
| —(C=O)O—CH(C <sub>6</sub> H <sub>5</sub> ) <sub>2</sub>                             | diphenylmethoxycarbonyl                      |
| —(C=O)O—C(C <sub>6</sub> H <sub>5</sub> ) <sub>3</sub>                              | triphenylmethoxycarbonyl                     |
| —(C=O)O—C <sub>6</sub> H <sub>5</sub>                                               | phenoxy carbonyl                             |
| 60   —(C=O)O—C <sub>6</sub> H <sub>4</sub> NO <sub>2</sub>                          | p-nitrophenoxycarbonyl                       |
| —(C=O)O—C <sub>6</sub> H <sub>4</sub> CH <sub>3</sub>                               | 3-methylphenoxycarbonyl                      |
| —(C=O)O—C <sub>6</sub> H <sub>3</sub> (CH <sub>3</sub> ) <sub>2</sub>               | 3,4-dimethylphenoxycarbonyl                  |
| —(C=O)O—C <sub>6</sub> H <sub>3</sub> (CH <sub>3</sub> ) <sub>2</sub>               | 3,5-dimethylphenoxycarbonyl                  |
| —(C=O)O—C <sub>6</sub> H <sub>4</sub> -sec-C <sub>4</sub> H <sub>9</sub>            | 2-sec-butylphenoxycarbonyl                   |
| 65   —(C=O)O—C <sub>10</sub> H <sub>7</sub>                                         | naphthylloxycarbonyl                         |



Since coloring temperature of the recording sheet of the present invention depends on a dissociation temperature of the blocked color developer, it is preferable that the blocked color developer has a low dissociation temperature. In view of dissociation temperature of the blocked color developer, it is preferable that the aromatic ring (R in Formula (1)) having blocked phenolic hydroxyl groups with a color developing function has an electrophilic substituent or residue. In other words, the aromatic ring having phenolic hydroxyl groups with a color developing function has an electrophilic substituent or residue, and at least one of the color developing phenolic hydroxyl groups is blocked by O-substituted oxycarbonyl group. That is, a color developer of Formula (2) is more preferable.



(wherein R<sub>1</sub>, a and b are the same as those in Formula (1). R<sub>2</sub> denotes a substituted or unsubstituted C<sub>6</sub>~C<sub>30</sub>-aromatic ring, and c is an integer from 1 to 4. X is halogen atom, nitoro group, substituted or unsubstituted C<sub>1</sub>~C<sub>18</sub>-alklamino group, carboxyl group, —C(=O)OY, —C(=O)NHY, or —SO<sub>2</sub>Y, Y is substituted or unsubstituted C<sub>1</sub>~C<sub>18</sub>-alkyl group, substituted or unsubstituted C<sub>6</sub>~C<sub>20</sub>-aryl group, substituted or unsubstituted C<sub>6</sub>~C<sub>30</sub>-alkoxyaryl group, substituted or unsubstituted C<sub>6</sub>~C<sub>30</sub>-alkylcarbonyloxyaryl group, or substituted or unsubstituted C<sub>7</sub>~C<sub>18</sub>-arylalkyl group.)

Further, in view of the dissociation temperature, R<sub>1</sub> of the O-substituted oxycarbonyl group (—(C=O)OR<sub>1</sub>) of Formulae (1) and (2) is preferable to be such that the cation is stable but easy to dissociate such as tertiary carbo-cation or benzyl-cation. Specifically, tert-butyl, benzyl, p-nitrobenzyl,  $\alpha$ -nitrobenzyl,  $\alpha$ -methylbenzyl,  $\alpha, \alpha$ -dimethylbenzyl, diphenylmethyl, or triphenylmethyl group is preferable. In addition, an electrophilic substituent or a substituent having an electrophilic substituent such as halogenated alkyl group (for example, chloromethyl group, dichloromethyl group, trichloromethyl group, trifluoromethyl group, or trichloro methyl group) is also preferable. That is the following color developer of Formula (3) is more preferable.



(wherein a and b are the same as those in Formula (1), and R<sub>2</sub>, X, and c are the same as those in Formula (2). R<sub>3</sub> is tert-butyl group, substituted or unsubstituted C<sub>1</sub>~C<sub>6</sub> halogenated alkyl group, benzyl group, p-nitrobenzyl group,  $\alpha$ -methylbenzyl,  $\alpha$ ,  $\alpha$ -dimethylbenzyl group, diphenylmethyl group, triphenylmethyl group.)

As the blocked color developer, Formulae (4), (5), (6), and (7) are more preferable.



(wherein R<sub>4</sub> and R<sub>5</sub> denote a substituted or unsubstituted C<sub>6</sub>~C<sub>20</sub>-aromatic ring, and R<sub>4</sub> and R<sub>5</sub> may be the same or different. R<sub>3</sub> is the same as that in Formula (3). R<sub>6</sub> denotes substituted or unsubstituted C<sub>1</sub>~C<sub>18</sub>-alkyl group, substituted or unsubstituted C<sub>6</sub>~C<sub>30</sub>-alkylaryl group, substituted or unsubstituted C<sub>6</sub>~C<sub>30</sub>-alkoxyaryl group, substituted or unsubstituted C<sub>6</sub>~C<sub>30</sub>-halogenated aryl group, or substituted or unsubstituted C<sub>10</sub>~C<sub>30</sub>-naphthyl group.)



(wherein R<sub>3</sub> is the same as that in Formula (3). R<sub>7</sub> is substituted or unsubstituted C<sub>1</sub>~C<sub>20</sub>-alkyl group).

Practical examples of the carbonate type blocked color developer include those compounds as described in Japanese OPI 5-177950.



-continued



-continued



-continued



-continued



-continued



However, by protecting the hydroxyl group, it is possible to widely select organic metal salts, inorganic metal salts, and leuco dyes.

Organic acid used in the organic metal salts of the present invention include benzoic acid compounds such as o-benzoylbenzoic acid, o-alkyl substituted benzoylbenzoic acid, o-alkylbenzoic acid, m-alkylbenzoic acid, o-tolylbenzoic acid, m-tolylbenzoic acid, o-halogenated benzoic acid, and m-halogenated benzoic acid; and fatty acids such as acetic acid, propionic acid, stearic acid, behenic acid, and palmitic acid. Metal elements in the metal salts of organic acids include iron, zinc, silver, copper, tin, calcium, magnesium, aluminum, barium, manganese, nickel, vanadium, cobalt, titanium, tungsten, mercury, and the like. In the present invention, iron-salt is preferable.

The metal salts of inorganic acids include ferric chloride, ferric sulfate, ammonium vanadate, and the like.

The leuco dye used in the present invention can be any type of electron-donating colorless dyes known in the area of conventional pressure-sensitive or thermal recording paper. Typical types are shown below:

3,3-Bis (4'-dimethylaminophenyl)-6-dimethylaminophthalide (Crystal Violet Lactone)  
 3,3-Bis(4'-dimethylaminophenyl)phthalide (Malachite Green Lactone)  
 Tris[4-(dimethylamino)phenyl]methane (Leuco Crystal Violet)  
 3-Diethylamino-6-methylfluorane  
 3-Diethylamino-7-methylfluorane  
 3-Diethylamino-7-chlorofluorane  
 3-Diethylamino-6-methyl-7-chlorofluorane  
 3-Diethylamino-6-chloro-7-methylfluorane  
 3-Diethylamino-6-methyl-7-anilinofluorane  
 3-Diethylamino-6-methyl-7-p-methylanilinofluorane  
 3-Diethylamino-6-methyl-7-(o,p-dimethylanilino)fluorane  
 3-Diethylamino-6-methyl-7-(m-trifluoromethylanilino)fluorane  
 3-Diethylamino-7-(o-chloroanilino)fluorane  
 3-Diethylamino-7-(p-chloroanilino)fluorane  
 3-Diethylamino-6-methyl-7-(o-chloroanilino)fluorane  
 3-Diethylamino-6-methyl-7-(p-chloroanilino)fluorane

- 25 3-Diethylamino-6-methyl-7-(o-fluoranilino)fluorane  
 3-Diethylamino-6-methyl-7-n-octylanilinofluorane  
 3-Diethylamino-6-methyl-7-benzylanilinofluorane  
 3-Diethylamino-6-methyl-7-dibenzylanilinofluorane  
 3-Diethylamino-benzo[a]fluorane  
 30 3-Diethylamino-benzo[c]fluorane  
 3-Dibutylamino-6-methyl-7-anilinofluorane  
 3-Dibutylamino-6-methyl-7-p-methylanilinofluorane  
 3-Dibutylamino-6-methyl-7-(o-chloroanilino)fluorane  
 3-Dibutylamino-6-methyl-7-(p-chloroanilino)fluorane  
 35 3-Dibutylamino-6-ethoxyethyl-7-anilinofluorane  
 3-Dibutylamino-6-ethoxyethyl-7-anilinofluorane  
 3-Di-n-pentylamino-7-(o-chloroanilino)fluorane  
 3-Di-n-pentylamino-6-methyl-7-(o-chloroanilino)fluorane  
 3-Pyrrolidyl-6-methyl-7-anilinofluorane  
 40 3-Piperidyl-6-methyl-7-anilinofluorane  
 3-(N-ethyl-N-isoamylamino)-6-methyl-7-anilinofluorane  
 3-(N-ethyl-N-isoamylamino)-6-chloro-7-anilinofluorane  
 3-(N-ethyl-N-cyclohexyl)-6-methyl-7-anilinofluorane  
 2-(4-Oxaheyl)-3-diethylamino-6-methyl-7-anilinofluorane  
 45 3,6,6'-Tris(dimethylamino)spiro[fluorene-9,3'-phthalide]  
 3-(4-Diethylamino-2-ethoxyphenyl)-3-(1-ethyl-2-methylin-dol-3-yl)-4-azaphthalide  
 3-(4-Diethylamino-2-ethoxyphenyl)-3-(1-octyl-2-methylin-dol-3-yl)-4-azaphthalide  
 50 3-(4-Cyclohexylethylamino-2-methoxyphenyl)-3-(1-ethyl-2-methylin-dol-3-yl)-4-azaphthalide  
 3,3-Bis(1-ethyl-2-methylin-dol-3-yl)phthalide  
 3,6-Bis(diethylamino)fluorane-γ-(3'-nitro)anilinofluorane  
 3,6-Bis(diethylamino)fluorane-γ-(4'-nitro)anilinofluorane  
 55 These dyes can be used alone or in combination. Furthermore, dyes which have heretofore been difficult to use due to liability to fogging can also be used.
- The binder can be cellulose derivatives such as hydroxyethylcellulose, carboxymethylcellulose, methylcellulose, and ethylcellulose; starch and its derivatives; gelatine, caseine, polyvinylalcohol, sodium polyacrylate, denatured polyvinylalcohol such as fully saponified polyvinylalcohol, partially saponified polyvinylalcohol, carboxylated polyvinylalcohol, polyvinylbutyral; sodium polyacrylate, polyethyleneoxide, acrylamide-acrylic ester copolymer, styrene-maleic anhydride copolymer, polyacrylamide, sodium

alginate, gelatin, casein, polystyrene, polyvinylacetate, polyurethane, polyacrylic acid, polyacrylic esters, styrene-butadiene copolymer, acrylonitrile-butadiene copolymer, vinylchloride-vinylacetate copolymer, styrene-butadiene-acrylic copolymer, and the like.

Among these, polyvinylalcohol type binders are more preferable in terms of dispersibility and the like. These binders are used by dissolving in water, alcohol, ketone, esters, hydrocarbons, or the like, or dispersing in water or other solvents, or dispersing in the form of a paste, and may be used as necessary.

The substrate can be paper, synthetic paper, non-woven fabrics, metallic foils, plastic films, plastic sheet, or the like, and composite sheets thereof may be used.

In the present invention, a sensitized, organic or inorganic fillers, waxes, an antisticking agent, an ultraviolet absorber, an antioxidant, a water-resistant agent, a dispersant, a defoamer, a fluorescent dye, and the like can be mixed in the recording layer as necessary.

As the sensitizer, any type of thermally fusible organic compounds known as sensitizers in the area of thermal recording can be used. Such sensitizers include:

Stearamide  
Palmitamide  
Ethylenebisamide  
1,2-Diphenoxymethane  
1,2-Di(3-methylphenoxy)ethane  
p-Benzylbiphenyl  
4-Biphenyl-p-tolylether  
m-Terphenyl  
Dibenzyl oxalate  
Di(p-chlorobenzyl) oxalate  
Di(p-methylbenzyl) oxalate  
Benzyl terephthalate  
Benzyl p-bezoxybenzoate

Prior art sensitizers in the area of thermal recording are lower in melting point than the leuco dyes and color developers; the sensitizer first melts by heat, and then the molten sensitizer dissolves with the leuco dye or the color developer to decrease the coloring start temperature. On the other hand, in the present invention, the coloring start temperature depends mainly on the decomposition temperature of the blocked color developer, the sensitizer melts to mix the color developer with the coloring substance homogeneously.

The organic or inorganic fillers include silica, kaolin, calcined kaolin, diatomaceous earth, talc, calcium carbonate, magnesium carbonate, titanium oxide, zinc oxide, aluminum hydroxide, urea-formaldehyde resin, styrene-methacrylic acid copolymer, styrene-butadiene copolymer, polystyrene resin, and the like.

The types and amounts of the blocked color developer, the metal salt of organic acid, the inorganic metal salt or leuco dye, the binder, and other ingredients are determined according to the properties required and recording characteristics and not specifically limited but, normally, 1 to 10 parts of the blocked color developer, 0.5 to 5 parts of the metal salt of organic acid, the inorganic metal salt or leuco dye, and 0.5 to 10 in the total solids of the binder are used, and 2 to 15 parts of the filler is preferably used.

The recording sheet of the present invention can be provided on the recording layer with an overcoat layer comprising a polymeric substance to enhance the storage stability, or under the recording layer with an undercoat layer comprising a filler-containing polymeric substance to enhance the coloring sensitivity.

Since the recording sheet of the present invention is very high in the background color stability, it is possible to heat laminate with a plastic film to provide a transparent and strong protective film. For example, heat-resistant cards can be easily produced using a commercial laminate machine. Further, the recording surface can be toner recorded.

To obtain an optical recording sheet, a dispersion comprising a sensitizer containing a light absorbent dispersed with a binder is mixed with the above dispersions to obtain an opaque undeveloped coating color for optical recording sheet. The coating color is coated on the substrate and dried to obtain an optical recording sheet.

The light absorbent used in the optical recording sheet of the present invention can be a substance which absorbs wavelengths of various light sources, and various types of dyes, pigments, near-infrared absorbents, and the like can be used.

Specifically, when a stroboflash lamp or the like is used as a recording light source (continuous wavelength), light absorbents are heat reaction products of thiourea derivative/cooper compounds described in Japanese OPI 2-206583 and Japanese Patent Application 5-30954 (Japanese Patent Publication Laid-open 5-199664), graphite, copper sulfide, molybdenum trisulfide, titanium black, carbon black, and like.

When a semiconductor laser and the like is used as a recording light source (single wavelength), the light absorbent can be immonium or diimmonium compounds such as IRGOO2 (Nippon Kayaku) or IRGO22 (Nippon Kayaku); dithiolatenickel complexes such as bisdithiobenzilnickel complex, toluenedithiolnickel complex, or 4-tert-butyl-1,2-benzenedithiolnickel complex; cyanine type dyes such as Indocyanine Green (Dia-ichi Seiyaku), NK-2014 (Nippon Kanko Shikiso Kenkyusho), NK-2612 (Nippon Kanko Shikiso Kenkyusho), 1,1,5,5-tetrakis(p-dimethylaminophenyl)-3-methoxy-1,4-pentadienotoluene, 1,1,5,5-tetrakis(p-diethylaminophenyl)-3-methoxy-1,4-pentadienotoluene; squalylium type dyes such as NK-2772 (Nippon Kanko Shikiso Kenkyusho); naphtoquinone type dyes, phthalocyanine type dyes, naphthoquinone type dyes, or anthraquinone type dyes. These light absorbents can also be used in combination.

Recording to the optical recording sheet is preferably achieved by a laser, rather than by a thermal head, using a semiconductor laser of several tens of mW.

The resulting recording sheet is also useful as a recording material which is superior in heat resistance and solvent resistance, or as a high-temperature thermolabel utilizing a specific temperature at which the blocked group dissociates.

In the thus obtained recording sheet, the blocked group of the blocked color developer is dissociated by way of light or heat to reveal a color developing function, and immediately reacts with the metal salt or leuco dye to develop a color. Therefore, the recording sheet of the present invention does not develop a color unless the blocked group of the blocked color developer dissociates, and does not cause unnecessary coloring by heat or solvents. Further, the carbonate type blocked color developer, when the blocked group dissociates by heating is considered to decompose to a color developing compound, carbon dioxide, and a compound derived from O-substituent of the O-substituted oxycarbonyl group, and is thus relatively high in safety.

Furthermore, the resulting recording sheet, when thermally recorded by a thermal head, tends to be difficult to give a sharp image in high-speed recording depending on the energy applied, due to difficulty in dissociation of the blocked group. On the other hand, the optical recording sheet containing a light absorbent can be recorded in a high density by irradiation of laser light because laser irradiation can be higher in energy density than a thermal head.

### DESCRIPTION OF PREFERRED EMBODIMENTS

#### Production of the blocked color developer

Compounds (8) to (23) were synthesized by the following method:



Melting point was measured by thermoanalysis (SSC5200 System (Seiko Denshi)). Melting points were not noted in Synthesis Examples 1, 3, and 12.

#### Synthesis Example 1

(11) (synthesis of Compound (8))  
n-Propyl gallate in an amount of 5.3 g (25 mM) was dissolved in ethyl acetate (25 ml), and then mixed with 23 ml (100 mM) of di-tert-butyl dicarbonate and pyridine (2 ml). The solution was reacted at 50° C. for 2.5 hours in a nitrogen atmosphere. The reaction solution was diluted with ethyl acetate, washed with 6% sodium hydroxide solution, 1N hydrochloric acid, and brine dried with anhydrous sodium sulfate, and the solvent was distilled out. The resulting oily substance was crystallized from n-hexane. The product was identified by means of <sup>1</sup>H-NMR to be n-propyl gallate tri-tert-butyl carbonate. (Yield: 67.2%)

Melting point: 60° C. <sup>1</sup>H-NMR: 0.94 (3H, t, J=7.5), 1.47 (27H, s), 1.67–1.74 (2H, m), 4.20 (2H, t, J=6.6), 7.77 (2H, s).

#### Synthesis Example 2

(14) (Synthesis of compound (9))  
n-Propyl gallate in an amount of 1.06 g (5 mM) was dissolved in ethyl acetate (20 ml), and then mixed with 5.7 ml (25 mM) of di-tert-butyl dicarbonate and pyridine (2 ml). The solution was reacted at room temperature for 2.5 hours

## 21

in a nitrogen atmosphere. The reaction solution was treated using the same procedure as in Synthesis Example 1. The resulting oily substance was purified by a silica gel column (developing solution: ethyl acetate/n-hexane (v/v=1:2)). The product was identified by means of  $^1\text{H-NMR}$  to be n-propyl gallate di-tert-butylcarbonate. (Yield: 50.4%)

$^1\text{H-NMR}$ : 1.01 (3H, t,  $J=7.0$ ), 1.56 (18H, s), 1.74–1.81 (2H, m) 4.24 (2H, t,  $J=7.0$ ), 7.79 (2H, s).

## Synthesis Example 3

## (Synthesis of compound (10))

n-Propyl gallate in an amount of 1.06 g (5 mM) was dissolved in ethyl acetate (20 ml), and then mixed with 1.9 ml (25 mM) of methyl chloroformate and pyridine (2 ml). The solution was reacted at 50° C. for 3 hours in a nitrogen atmosphere. The reaction solution was treated using the same procedure as in Synthesis Example 2 to obtain n-propyl gallate trimethylcarbonate. (Yield: 60.2%)

$^1\text{H-NMR}$ : 1.01 (3H, t,  $J=7.4$ ), 1.78 (2H, m), 3.92 (3H, s), 3.93 (6H, s), 4.28 (2H, t,  $J=7.4$ ), 7.91 (2H, s).

## Synthesis Example 4

## Synthesis of compound (11))

n-Propyl gallate in an amount of 1.06 g (5 mM) was dissolved in ethyl acetate (20 ml), and then mixed with 2.5 ml (20 mM) of phenyl chloroformate and pyridine (1 ml). The solution was reacted at 50° C. for 3 hours in a nitrogen atmosphere. The reaction solution was treated using the same procedure as in Synthesis Example 2 to obtain n-propyl gallate triphenylcarbonate. (Yield: 58.6%)

Melting point: 99° C.  $^1\text{H-NMR}$ : 1.02 (3H, t,  $J=7.0$ ), 1.80 (2H, dd,  $J=14.0, 7.1$ ), 4.30 (2H, t,  $J=6.7$ ), 7.23–7.44 (15H, m), 8.08 (2H, s).

## Synthesis Example 5

(Synthesis of compound (12)) 4-Hydroxy-4'-isopropoxydiphenylsulfone in an amount of 1.17 g (4 mM) was dissolved in ethyl acetate (7 ml), and pyridine (0.65 ml). The solution was reacted at 50° C. for 30 minutes in a nitrogen atmosphere. The reaction solution was treated using the same procedure as in Synthesis Example 1 to obtain 4ethoxycarbonyloxy-4'-isopropoxydiphenylsulfone. (Yield: 93.7%)

Melting point: 88° C.  $^1\text{H-NMR}$ : 1.33 (3H, s), 1.35 (3H, s), 1.39 (3H, t,  $J=6.5$ ), 4.33 (2H, dd,  $J=14.0, 6.5$ ), 4.61 (1H, ddd,  $J=12.0, 6.1, 6.0$ ), 6.93 (2H, d,  $J=10.0$ ), 7.31 (2H, d,  $J=9.5$ ), 7.84 (2H, d,  $J=10.0$ ), 7.95 (2H, d,  $J=9.5$ ).

## Synthesis Example 6

Synthesis of compound (13)) 4-Hydroxy-4'-isopropoxydiphenylsulfone in an amount of 1.17 g (4 mM) was dissolved in ethyl acetate (7 ml), and then mixed with 0.79 ml (6 mM) of iso-butyl chloroformate and pyridine (0.65 ml). The solution was reacted at 50° C. for 1 hour in a nitrogen atmosphere. The reaction solution was treated using the same procedure as in Synthesis Example 1 to obtain 4-iso-butoxycarbonyloxy-4'-isopropoxydiphenylsulfone. (Yield: 75.8%)

Melting point: 81° C.  $^1\text{H-NMR}$ : 0.98 (3H, s), 1.00 (3H, s), 1.33 (3H, s), 2.00–2.11 (1H, m), 4.04 (2H, d,  $J=6.5$ ), 4.57–4.65 (1H, m), 6.93 (2H, d,  $J=9.0$ ), 7.31 (2H, d,  $J=9.0$ ), 7.84 (2H, d,  $J=9.0$ ), 7.95 (2H, d,  $J=9.0$ ).

## 22

## Synthesis Example 7

## (Synthesis of compound (14))

4-Hydroxy-4'-isopropoxydiphenylsulfone in an amount of 1.75 g (6 mM) was dissolved in ethyl acetate (10 ml), and then mixed with 1.6 ml (7.2 mM) of di-tert-butyldicarbonate and pyridine (2 ml). The solution was reacted at 50° C. for 3 hours in a nitrogen atmosphere. The reaction solution was treated using the same procedure as in Synthesis Example 1. The product was identified by means of  $^1\text{H-NMR}$  to be 4-tert-butoxycarbonyloxy-4'-isopropoxydiphenylsulfone.

Melting point: 105° C.  $^1\text{H-NMR}$ : 1.33 (3H, s), 1.35 (3H, s), 1.55 (9H, s), 4.60 (1H, m), 6.92 (2H, d,  $J=8.5$ ), 7.29 (2H, d,  $J=8.5$ ), 7.83 (2H, d,  $J=8.5$ ), 7.94 (2H, d,  $J=8.5$ ).

## Synthesis Example 8

## (Synthesis of compound (15))

4-Hydroxy-4'-isopropoxydiphenylsulfone in an amount of 1.17 g (4 mM) was dissolved in ethyl acetate (7 ml), and then mixed with 0.97 ml (5 mM) of 2-ethylhexyl chloroformate and pyridine (0.5 ml). The solution was reacted at 50° C. for 3 hours in a nitrogen atmosphere. The reaction solution was treated using the same procedure as in Synthesis Example 1 to obtain 4-(2-ethylhexyloxy)carbonyloxy-4'-isopropoxydiphenylsulfone as a colorless oily substance. (Yield: 50%)

$^1\text{H-NMR}$ : 0.90 (3H, t,  $J=7.0$ ), 0.92 (3H, t,  $J=7.5$ ), 1.30–1.40 (15H, m), 4.18 (2H, dd,  $J=6.0, 1.5$ ), 4.61 (1H, ddd,  $J=11.5, 6.0, 6.0$ ), 6.93 (2H, d,  $J=9.0$ ), 7.31 (2H, d,  $J=9.0$ ), 7.84 (2H, d,  $J=9.0$ ), 7.94 (2H, d,  $J=9.0$ ).

## Synthesis Example 9

## (Synthesis of compound (16))

4-Hydroxy-4'-isopropoxydiphenylsulfone in an amount of 1.17 g (4 mM) was dissolved in ethyl acetate (7 ml), and then mixed with 0.62 ml (6 mM) of 2-chloroethyl chloroformate and pyridine (0.65 ml). The solution was reacted at 50° C. for 1 hour in a nitrogen atmosphere. The reaction solution was treated using the same procedure as in Synthesis Example 1 to obtain 4-(2-chloroethoxy) carbonyloxy-4'-isopropoxydiphenylsulfone. (Yield: 90.3%)

Melting point: 111° C.  $^1\text{H-NMR}$ : 1.33 (3H, s), 1.35 (3H, s), 3.78 (2H, t,  $J=6.0$ ), 4.51 (2H, t,  $J=6.0$ ), 4.61 (1H, dt,  $J=12.0, 6.0$ ), 6.93 (2H, d,  $J=9.0$ ), 7.32 (2H, d,  $J=9.0$ ), 7.84 (2H, d,  $J=9.0$ ), 7.95 (2H, d,  $J=9.0$ ).

## Synthesis Example 10

## (Synthesis of compound (17))

4-Hydroxy-4'-isopropoxydiphenylsulfone in an amount of 1.17 g (4 mM) was dissolved in ethyl acetate (7 ml), and then mixed with 0.80 ml (6 mM) of 2,2,2-trichloroethyl chloroformate and pyridine (0.65 ml). The solution was reacted at 50° C. for 1 hour in a nitrogen atmosphere. The reaction solution was treated using the same procedure as in Synthesis Example 1 to obtain 4-(2,2,2-trichloroethoxy)carbonyloxy-4'-isopropoxydiphenylsulfone. (Yield: 28.7%)

Melting point: 103° C.  $^1\text{H-NMR}$ : 1.33 (3H, s), 1.36 (3H, s), 4.57–4.65 (1H, m), 6.94 (2H, d,  $J=9.0$ ), 7.37 (2H, d,  $J=9.0$ ), 7.85 (2H, d,  $J=9.0$ ), 7.98 (2H, d,  $J=9.0$ ).

## Synthesis Example 11

## (Synthesis of compound (18))

4-Hydroxy-4'-isopropoxydiphenylsulfone in an amount of 1.17 g (4 mM) was dissolved in ethyl acetate (5 ml), and then mixed with 3.6 ml of toluene solution (30–35%) of

## 23

benzyl chloroformate and pyridine (0.65 ml). The solution was reacted at 50° C. for 3 hours in a nitrogen atmosphere. The reaction solution was treated using the same procedure as in Synthesis Example 1 to obtain 4-benzylxycarbonyloxy-4'-isopropoxydiphenylsulfone. (Yield: 74.3%)

Melting point: 119° C.  $^1\text{H-NMR}$ : 1.33 (3H, s), 1.35 (3H, s), 4.61 (1H, ddd,  $J=12.0, 6.0, 6.0$ ), 5.26 (2H, s), 6.86–6.92 (1H, m), 6.93 (2H, d,  $J=10.0$ ), 7.31 (2H, d,  $J=9.5$ ), 7.36–7.44 (4H, m), 7.83 (2H, d,  $J=9.5$ ), 7.98 (2H, d,  $J=10.0$ ).

## Synthesis Example 12

## (Synthesis of compound (19))

Bis(4-hydroxyphenyl)sulfone in an amount of 1.0 g (4 mM) was dissolved in ethyl acetate (10 ml), and then mixed with 2.7 ml (12 mM) of di-tert-butyldicarbonate and pyridine (1 ml). The solution was reacted at 50° C. for 3 hours in a nitrogen atmosphere. The reaction solution was treated using the same procedure as in Synthesis Example 1. The product was identified by means of  $^1\text{H-NMR}$  to be di-tert-butyldicarbonate of bis(4-hydroxyphenyl)sulfone. (Yield: 73.6%)

$^1\text{H-NMR}$ : 1.55 (18H, s), 7.32 (4H, d,  $J=8.0$ ), 7.95 (4H, d,  $J=8.0$ ).

## Synthesis Example 13

## (Synthesis of compound (20))

Bisphenol A in an amount of 2.28 g (10 mM) was dissolved in ethyl acetate (10 ml), and then mixed with 6.9 ml (30 mM) of di-tert-butyldicarbonate and pyridine (1 ml). The solution was reacted at 50° C. for 3 hours in a nitrogen atmosphere. The reaction solution was treated using the same procedure as in Synthesis Example 1. The product was identified by means of  $^1\text{H-NMR}$  to be bisphenol A with its hydroxyl group blocked by di-tert-butoxycarbonyl group. (Yield: 60.9%)

Melting point: 103° C.  $^1\text{H-NMR}$ : 1.55 (18H, s), 1.65 (6H, s), 7.05 (4H, d,  $J=8.5$ ), 7.21 (4H, dt,  $J=8.5$ ).

## Synthesis Example 14

## (Synthesis of compound (21))

4,4'-Thiodiphenol in an amount of 0.87 g (4 mM) was dissolved in ethyl acetate (10 ml), and then mixed with 2.7 ml (12 mM) of di-tert-butyldicarbonate and pyridine (1 ml). The solution was reacted at 50° C. for 3 hours in a nitrogen atmosphere. The reaction solution was treated using the same procedure as in Synthesis Example 1 to obtain di-tert-butyldicarbonate of 4,4'-thiodiphenol. (Yield: 66.6%)

Melting point: 131° C.  $^1\text{H-NMR}$ : 1.55 (18H, s), 7.11 (4H, d,  $J=8.6$ ), 7.33 (4H, dt,  $J=8.6$ ).

## Synthesis Example 15

## (Synthesis of compound (22))

Methyl bis(4-hydroxyphenyl)acetate in an amount of 1.0 g (4 mM) was dissolved in ethyl acetate (10 ml), and then mixed with 2.7 ml (12 mM) of di-tert-butyldicarbonate and pyridine (1 ml). The solution was reacted at 50° C. for 2.5 hours in a nitrogen atmosphere. The reaction solution was treated using the same procedure as in Synthesis Example 1 to obtain di-tert-butyldicarbonate of methyl bis(4-hydroxyphenyl)acetate. (Yield: 79.9%)

Melting point: 140° C.  $^1\text{H-NMR}$ : 1.55 (18H, s), 3.73 (3H, s), 5.00 (1H, s), 7.12 (4H, d,  $J=8.0$ ), 7.30 (4H, dt,  $J=8.6$ ).

## 24

## Synthesis Example 16

## (Synthesis of compound (23))

Benzyl p-hydroxybenzoate in an amount of 0.9 g (4 mM) was dissolved in ethyl acetate (10 ml), and then mixed with 2.7 ml (12 mM) of di-tert-butyldicarbonate and pyridine (1 ml). The solution was reacted at 50° C. for 2.5 hours in a nitrogen atmosphere. The reaction solution was treated using the same procedure as in Synthesis Example 1 to obtain benzyl p-(tert-butoxycarbonyloxy)benzoate. (Yield: 39.6%)

Melting point: 81° C.  $^1\text{H-NMR}$ : 1.55 (9H, s), 5.36 (2H, s), 7.25 (2H, d,  $J=9.0$ ), 7.31–7.47 (5H, m), 8.10 (2H, d,  $J=9.0$ ). Production of recording sheet

## EXAMPLE 1

A metal salt dispersion (solution A) of the composition shown below and a dispersion (solution B) of the blocked color developer of Synthesis Example 1 were individually wet pulverized for 1 hour by a sand grinder.

## Solution A: (metal salt dispersion)

|                                       |           |
|---------------------------------------|-----------|
| Iron behenate                         | 4.0 parts |
| 10% Aqueous polyvinylalcohol solution | 10.0      |
| Water                                 | 6.0       |

## Solution B: (blocked color developer dispersion)

|                                                |           |
|------------------------------------------------|-----------|
| Blocked color developer of Synthesis Example 1 | 4.0 parts |
| Zinc stearate                                  | 1.5       |
| 10% Aqueous polyvinylalcohol solution          | 13.75     |
| Water                                          | 8.25      |

Then, 20 parts of the solution A, 36.5 parts of the solution B, and 12 parts of a 50% aqueous dispersion of silica were mixed to obtain a coating color. The coating color was coated on fine paper with a substance of 60 g/m<sup>2</sup> using a Meyer bar, and dried to obtain an optical recording sheet with a coating coverage of 6 g/m<sup>2</sup>.

The recording sheet was printed by a label printer of the TEC Electronic Fee-Charging Scale HP-9303 (Tokyo Denki) to obtain a print.

## EXAMPLE 2

A dispersion (solution C) of light absorbent sensitizer of the composition shown below was wet pulverized for 1 hour by a sand grinder. (optical density—1.28(measured by RD-914)) Solution C: (light absorbent dispersion)

p-Benzylbiphenyl (PBB) in an amount of 49 parts was mixed with 1 part of toluenedithiolnickel complex, heated to 100°–150° C. to melt, and pulverized by a sand grinder to obtain a light absorbent sensitizer.

|                                       |           |
|---------------------------------------|-----------|
| Light absorbent sensitizer            | 4.0 parts |
| 10% Aqueous polyvinylalcohol solution | 10.0      |
| Water                                 | 6.0       |

Then, 10 parts of the solution A of Example 1, 42 parts of the solution B of Example 1, 20 parts of the solution C, 25 parts of 25% aqueous dispersion of silica, and 10 parts of a 10% aqueous polyvinylalcohol solution were mixed to obtain a coating color. The coating color was coated on fine paper with a substance of 60 g/m<sup>2</sup> using a Meyer bar, and

## 25

dried to obtain an optical recording sheet with a coating coverage of 6 g/m<sup>2</sup>.

The recording sheet was irradiated with laser light by a laser plotter described in Japanese OPI 03-239598 to obtain a clear print.

## EXAMPLE 3

The same procedure as in Example 2 was used, except that a dispersion (solution D) of leuco dye of the following composition was used in place of the solution A of Example 1, to obtain an optical recording sheet.

| Solution D: (leuco dye dispersion)    |           |
|---------------------------------------|-----------|
| ODB                                   | 2.0 parts |
| 10% Aqueous polyvinylalcohol solution | 3.4       |
| Water                                 | 1.9       |

\*ODB=3-diethylamino-6-methyl-7-anilinofluorane

The recording sheet was irradiated with laser light as in Example 2 to obtain a clear print.

## EXAMPLE 4

The same procedure as in Example 2 was used, except that iron o-benzoylbenzoate was used in place of the iron behenate in the metal salt dispersion (solution A) of Example 1, to obtain an optical recording sheet.

The recording sheet was irradiated with laser light as in Example 2 to obtain a clear print.

## EXAMPLE 5

The same procedure as in Example 2 was used, except that dithiobenzilnickel complex was used in place of the toluenedithiobenzilnickel complex in the light absorbent sensitizer dispersion (solution C) of Example 2, to obtain an optical recording sheet.

The recording sheet was irradiated with laser light as in Example 2 to obtain a clear print.

## EXAMPLE 6

The same procedure as in Example 2 was used, except that the blocked color developer of Synthesis Example 2 was used in place of the blocked color developer of Synthesis Example 1 in the blocked color developer dispersion (solution B) of Example 1, to obtain an optical recording sheet.

The recording sheet was irradiated with laser light as in Example 2 to obtain a clear print.

## EXAMPLE 7

The same procedure as in Example 2 was used, except that the blocked color developer of Synthesis Example 3 was used in place of the blocked color developer of Synthesis Example 1 in the blocked color developer dispersion (solution B) of Example 1, to obtain an optical recording sheet.

The recording sheet was irradiated with laser light as in Example 2 to obtain a clear print.

## EXAMPLE 8

The same procedure as in Example 2 was used, except that the blocked color developer of Synthesis Example 4 was used in place of the blocked color developer of Synthesis

## 26

Example 1 in the blocked color developer dispersion (solution B) of Example 1, to obtain an optical recording sheet.

The recording sheet was irradiated with laser light as in Example 2 to obtain a clear print.

## EXAMPLE 9

A dispersion (solution E) of blocked color developer of the composition shown below was pulverized for 1 hour by a sand grinder.

## Solution E: (blocked color developer dispersion)

|    |                                                |           |
|----|------------------------------------------------|-----------|
| 15 | Blocked color developer of Synthesis Example 5 | 6.0 parts |
|    | 10% Aqueous polyvinylalcohol solution          | 15.0      |
|    | Water                                          | 9.0       |

Then, 10 parts of the solution D of Example 3, 30 parts of the solution E, 20 parts of the solution C of Example 2, 25 parts of 25% aqueous dispersion of silica, and 10 parts of a 10% aqueous polyvinylalcohol solution were mixed to obtain a coating color. The coating color was coated on fine paper with a substance of 60 g/m<sup>2</sup> using a Meyer bar, and dried to obtain an optical recording sheet with a coating coverage of 6 g/m<sup>2</sup>.

The recording sheet was irradiated with laser light as in Example 2 to obtain a clear print.

## EXAMPLE 10

The same procedure as in Example 9 was used, except that the blocked color developer of Synthesis Example 6 was used in place of the blocked color developer of Synthesis Example 5 in the blocked color developer dispersion (solution B) of Example 1, to obtain an optical recording sheet.

The recording sheet was irradiated with laser light as in Example 2 to obtain a clear print.

## EXAMPLE 11

A dispersion (solution F) of blocked color developer of the composition shown below was pulverized for 1 hour by a sand grinder.

## Solution F: (blocked color developer dispersion)

|    |                                                |           |
|----|------------------------------------------------|-----------|
| 45 | Blocked color developer of Synthesis Example 7 | 6.0 parts |
|    | 10% Aqueous polyvinylalcohol solution          | 15.0      |
|    | Water                                          | 9.0       |

Then, 15 parts of the solution D of Example 3, 35 parts of the solution F, and 12 parts of 50% aqueous dispersion of silica were mixed to obtain a coating color. The coating color was coated on fine paper with a substance of 60 g/m<sup>2</sup> using a Meyer bar, and dried to obtain an optical recording sheet with a coating coverage of 6 g/m<sup>2</sup>.

The recording sheet was possible to be printed by the same method as in Example 1. (optical density=1.25)

## EXAMPLE 12

The same procedure as in Example 9 was used, except that the blocked color developer dispersion (solution F) of Synthesis Example 11 was used in place of the blocked color developer dispersion (solution E) of Synthesis Example 9, to obtain an optical recording sheet.

## 27

The recording sheet was irradiated with laser light as in Example 2 to obtain a clear print.

## EXAMPLE 13

The same procedure as in Example 12 was used, except that NK-2612 (Nippon Kanko Shikiso Kenkyusho) was used as a light absorbent in place of toluenedithiolnickel complex in the light absorbent sensitizer dispersion (solution C) of Example 2, to obtain an optical recording sheet.

The recording sheet was irradiated with laser light as in Example 2 to obtain a clear print.

## EXAMPLE 14

The same procedure as in Example 12 was used, except that 1,1,5,5-tetrakis-(p-dimethylaminophenyl)-3-methoxy-1,4-pentadiene was used as a light absorbent in place of toluenedithiolnickel complex in the light absorbent sensitizer dispersion (solution C) of Example 2, to obtain an optical recording sheet.

The recording sheet was irradiated with laser light as in Example 2 to obtain a clear print.

## EXAMPLE 15

The same procedure as in Example 12 was used, except that the blocked color developer of Synthesis Example 9 was used in place of the blocked color developer of Synthesis Example 7 in the blocked color developer dispersion (solution F) of Example 11, to obtain an optical recording sheet.

The recording sheet was irradiated with laser light as in Example 2 to obtain a clear print.

## EXAMPLE 16

The same procedure as in Example 12 was used, except that the blocked color developer of Synthesis Example 10 was used in place of the blocked color developer of Synthesis Example 7 in the blocked color developer dispersion (solution F) of Example 11, to obtain an optical recording sheet.

The recording sheet was irradiated with laser light as in Example 2 to obtain a clear print.

## EXAMPLE 17

The same procedure as in Example 12 was used, except that the blocked color developer of Synthesis Example 11 was used in place of the blocked color developer of Synthesis Example 7 in the blocked color developer dispersion (solution F) of Example 11, to obtain an optical recording sheet.

The recording sheet was irradiated with laser light as in Example 2 to obtain a clear print.

## EXAMPLE 18

The same procedure as in Example 11 was used, except that the blocked color developer of Synthesis Example 12 was used in place of the blocked color developer of Synthesis Example 7 in the blocked color developer dispersion (solution F) of Example 11, to obtain an optical recording sheet.

The recording sheet was irradiated with laser light as in Example 2 to obtain a clear print.

## 28

## EXAMPLE 19

The same procedure as in Example 11 was used, except that CVL was used in place of ODB in the leuco dye dispersion (solution D) of Synthesis Example 3, to obtain an optical recording sheet.

\*CVL=Crystal Violet Lactone

The recording sheet was possible to be printed by the same method as in Example 1. (optical density=0.88)

## EXAMPLE 20

A dispersion (solution G) of blocked color developer and a dispersion (solution H) of following composition were pulverized for 1 hour by a sand grinder.

## Solution G: (blocked color developer dispersion)

|                                                 |           |
|-------------------------------------------------|-----------|
| Blocked color developer of Synthesis Example 12 | 6.0 parts |
| 10% Aqueous polyvinylalcohol solution           | 15.0      |
| Water                                           | 9.0       |

## Solution H: (light absorbent sensitizer dispersion)

p-Benzylbiphenyl (PBB) in an amount of 48.4 parts was mixed with 1 part of toluenedithiolnickel complex and 0.6 part of NK-2612 (Nippon Kanko Shikiso Kenkyusho), heated to 100°-150° C. to melt, and treated by a sand grinder to obtain a light absorbent sensitizer.

|                                       |           |
|---------------------------------------|-----------|
| Light absorbent sensitizer            | 4.0 parts |
| 10% Aqueous polyvinylalcohol solution | 10.0      |
| Water                                 | 6.0       |

Then, 7.3 parts of the solution D of Example 3, 30 parts solution G, 20 parts of the solution H, 25 parts of 25% aqueous dispersion of silica, and 8 parts of 10% polyvinylalcohol were mixed to obtain a coating color. The coating color was coated on fine paper with a substance of 60 g/m<sup>2</sup> using a Meyer bar, and dried to obtain an optical recording sheet with a coating coverage of 6 g/m<sup>2</sup>.

The recording sheet was irradiated with laser light as in Example 2 to obtain a clear print.

## EXAMPLE 21

The same procedure as in Example 12 was used, except that the blocked color developer of Synthesis Example 13 was used in place of the blocked color developer of Synthesis Example 1 in the blocked color developer dispersion (solution B) of Example 1, to obtain an optical recording sheet.

The recording sheet was irradiated with laser light as in Example 2 to obtain a clear print.

## EXAMPLE 22

The same procedure as in Example 12 was used, except that the blocked color developer of Synthesis Example 14 was used in place of the blocked color developer of Synthesis Example 7 in the blocked color developer dispersion (solution F) of Example 11, to obtain an optical recording sheet.

The recording sheet was irradiated with laser light as in Example 2 to obtain a clear print.

## EXAMPLE 23

The same procedure as in Example 5 was used, except that the blocked color developer of Synthesis Example 15 was used in place of the blocked color developer of Synthesis Example 1 in the blocked color developer dispersion (solution B) of Example 1, to obtain an optical recording sheet.

The recording sheet was irradiated with laser light as in Example 2 to obtain a clear print.

## EXAMPLE 24

The same procedure as in Example 12 was used, except that the blocked color developer of Synthesis Example 16 was used in place of the blocked color developer of Synthesis Example 7 in the blocked color developer dispersion (solution F) of Example 11, to obtain an optical recording sheet.

The recording sheet was irradiated with laser light as in Example 2 to obtain a clear print.

## EXAMPLE 25

The same procedure as in Example 2 was used, except that ammonium vanadate was used in place of the iron behenate in the metal salt dispersion (solution A) of Example 1, to obtain a clear print.

The recording sheet was irradiated with laser light as in Example 2 to obtain a clear print.

## Comparative Example

The same procedure as in Example 1 was used, except that a color developer with phenolic hydroxyl group having a color developing function unblocked, that is, n-propyl gallate, was used in place of the blocked color developer of Synthesis Example 1 in the blocked color developer dispersion (solution B) of Example 1, to obtain an ordinary thermal recording sheet.

The ordinary thermal recording sheet underwent background coloring in a heat resistance test (80°C., 3 hours). However, no background coloring was noted in the recording sheet of the Example.

Further, in writing tests by an ink, background coloring was noted in the ordinary thermal recording sheet, whereas no change in background color was noted in the recording sheet of the Example.

Furthermore, when heat lamination was carried out using a pouch film by means of a Simple Lamination Apparatus (KS Pouch H-140: Meiko Shokai), the recording sheet of the Comparative Example underwent background coloring, whereas no change in background color was noted in the recording sheet according to the present invention.

As described above, with the blocked color developers of the present invention, since no coloring occurs as much as the blocked group of the blocked color developer does not dissociate, a recording sheet which is superior in solvent resistance and heat resistance to conventional recording sheets can be obtained. Further, with the blocked color developers of the present invention, the metal salt and leuco dye can be widely selected and, due to reduced coloring in dry state, production of the recording sheet is easy.

What is claimed is:

1. A recording sheet comprising an opaque recording layer containing a color developer of Formula (1) with at least one of phenolic hydroxyl groups having a color-

developing function blocked by an O-substituted oxycarbonyl group —(C=O)OR<sub>1</sub>, and a metal salt of an organic acid or a metal salt of an inorganic acid or a leuco dye reacting with said color developer to develop a color:



10 wherein R denotes a C<sub>6</sub> to C<sub>30</sub>-aromatic group, R<sub>1</sub> is a C<sub>1</sub> to C<sub>18</sub>-alkyl group, C<sub>3</sub> to C<sub>15</sub>-cycloalkyl group, C<sub>1</sub> to C<sub>12</sub>-halogenated alkyl group, C<sub>1</sub> to C<sub>12</sub>-silylalkyl group, vinyl group, allyl group, C<sub>7</sub> to C<sub>18</sub>-aryl alkyl group, C<sub>13</sub> to C<sub>25</sub>-diphenylmethyl group, C<sub>19</sub> to C<sub>35</sub>-triphenylmethyl group, C<sub>6</sub> to C<sub>20</sub>-aryl group, or C<sub>10</sub> to C<sub>20</sub>-naphthyl group, and a and b are each integers from 1 to 3, and a≥b.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9



wherein  $R_3$  is the same as that in Formula (3),  $R_7$  is  $C_6$  to  $C_{20}$ -alkyl group.

6. An optical recording sheet wherein a recording layer of the recording sheet of claim 1 contains a light absorbent for absorbing light and converting it to heat. 20

7. Recording cards comprising the recording sheet of claim 1, laminated with a plastic film.

8. A recording sheet comprising an opaque recording layer containing a color developer with at least one of phenolic hydroxyl groups having a color-developing function blocked by an O-substituted oxycarbonyl group  $-(C=O)OR_1$ , and a metal salt of an organic acid or a metal salt of an inorganic acid or a leuco dye reacting with said color developer to develop a color, said color developer having the formula 25



wherein  $X$  is  $C_3H_6$  or



$R_1$  is  $C_1$  to  $C_4$  alkyl or phenyl,  $a$  and  $b$  are each integers from 1 to 3, and  $a \geq b$ .

9. The recording sheet of claim 8 wherein in the color developer formula  $a$  is 3 and  $b$  is 2 or 3. 50

10. The recording sheet of claim 8 wherein in the color developer formula  $X$  is  $n-C_3H_7$  or iso- $C_3H_7$  and  $R_1$  is  $C_3-C_4$  n-alkyl or  $C_3-C_4$  iso-alkyl.

11. The recording sheet of claim 8 wherein the formula is 55



12. The recording sheet of claim 8 wherein the formula is



14. A recording sheet comprising an opaque recording layer containing a color developer and a metal salt of an organic acid or a metal salt of an inorganic acid or a leuco dye reacting with said color developer to develop a color, said color developer having the formula 20



wherein  $R_3$  is  $C_2$  to  $C_6$  alkyl or



15. A recording sheet comprising an opaque recording layer containing a color developer and a metal salt of an organic acid or a metal salt of an inorganic acid or a leuco dye reacting with said color developer to develop a color, wherein said color developer is a member selected from the group consisting of 40



60 65 wherein the  $R_1$  is  $C_2$  to  $C_6$  alkyl or phenyl.

16. The recording sheet of claim 15 wherein the color developer has the formula

33



17. The recording sheet of claim 15 wherein the color developer has the formula



18. The recording sheet of claim 15 wherein the color developer has the formula

5

10

15



19. The recording sheet of claim 15 wherein the color developer has the formula



\* \* \* \* \*